

Dec. 29, 1925.

1,567,574

N. S. CLAY

SPECIAL FABRIC PROPELLER

Filed Sept. 20, 1923



WITNESSES:

A. G. Schieffelin  
H. C. Biernan

INVENTOR

Noble S. Clay

BY  
B. Wesley Glare

ATTORNEY

Patented Dec. 29, 1925.

1,567,574

# UNITED STATES PATENT OFFICE.

NOBLE S. CLAY, OF WILKINSBURG, PENNSYLVANIA, ASSIGNOR TO WESTINGHOUSE ELECTRIC & MANUFACTURING COMPANY, A CORPORATION OF PENNSYLVANIA.

## SPECIAL FABRIC PROPELLER.

Application filed September 20, 1923. Serial No. 663,739.

To all whom it may concern:

Be it known that I, NOBLE S. CLAY, a citizen of the United States, and a resident of Wilkinsburg, in the county of Allegheny and State of Pennsylvania, have invented a new and useful Improvement in Special Fabric Propellers, of which the following is a specification.

My invention relates to propellers and more particularly to special fabric propellers for air craft.

Heretofore, various types of wooden propellers have been used, but it is becoming increasingly difficult to obtain the proper kind and grade of wood. The necessity of employing expert or skilled workmen, and the fact that wooden propellers warp and are subject to rapid wear, are important disadvantages. More recent developments have been to form a propeller from initially flexible material made rigid by the application of a binder which may be hardened, such as a phenolic condensation product.

In a process of this kind, the propeller is built up of laminations or layers of flexible material, pressed, molded or otherwise formed into the desired shape, such material being previously impregnated with a phenolic condensation product, so that when the assembled layers are heated under pressure the entire structure is compacted and rendered hard and substantially insoluble and it acquires a high degree of strength and rigidity.

Even such laminated propellers made as described above have been found to possess defects. Propellers of this type have more strength than is necessary, in a transverse direction and have been known to fail in the longitudinal direction. The strains and stresses set up by reason of centrifugal forces, bending and thrust moments and vibrations sometimes exceed the ultimate tensile strength of the material longitudinally.

My invention is intended to overcome the defects and disadvantages of previous structures as herein set forth, it being among the objects thereof to provide a propeller which shall have a high degree of strength in the direction of greatest strain.

In practicing my invention, I employ a special filling material and a phenolic condensation product or other binder which hardens and becomes substantially, infusible and insoluble upon the application of

heat, and, which is so designed as to resist longitudinal strains and stresses without sacrificing strength in the transverse direction. More specifically, I employ as a filling medium, laminations of cord fabric composed of relatively small transverse cords or strands, and tightly twisted cords which are relatively stronger and more numerous than the other or transverse cords or strands and a binder which hardens and becomes substantially infusible and insoluble upon the application of heat. The tightly twisted cords are placed longitudinally of the propeller blade.

I have found it preferable, however, to employ laminations of loose flat twisted longitudinal cords or strands which are relatively larger and more numerous than the transverse strands and a phenolic condensation product or other binder, which hardens and becomes substantially, insoluble and infusible upon the application of heat. This material provides a propeller structure which is considerably stronger than that formed from the ordinary cord fabric.

In the accompanying drawing constituting a part hereof and in which like reference characters represent like parts,

Figure 1 is a plan view of a propeller constructed in accordance with my invention;

Fig. 2 is a side elevational view thereof;

Fig. 3 is a sectional view along the line III—III of Fig. 2;

Fig. 4 is a sectional view along the line IV—IV Fig. 2;

Fig. 5 is a sectional view along the line II—II of Fig. 1 and shows the built up or laminated structure of the finished propeller, and

Fig. 6 is an enlarged, fragmentary plan view of the special fabric utilized.

The propeller 1 is preferably formed of a series of preformed layers or laminations 2, as generally shown in Figures 1-5. The layers or laminations 2 may be of special fabric or woven material composed of a plurality of classes of strands, so cut or formed that when forming the propeller, some of the strands 3, of which may be tightly twisted cords but preferably are loose, flat twisted cords, will be substantially parallel to the longitudinal axis of the propeller 1. The strands 3 are relatively larger, stronger and more numerous than the remaining strands 105 110

4 which are placed substantially transverse to the longitudinal axis of the propeller 1. The preferred structure of the special fabric is shown in Figures 3 and 4 and more in detail in the enlarged fragmentary view, Fig. 6. The strands or cords 3 are loose and flat twisted with filler strands or threads 4 of the same character.

The layers or laminations of special 10 fabric or woven material previously impregnated with a suitable binder are cut to the proper shapes and a suitable number thereof assembled in a mold. The cords 3 of each of the laminations 2 are substantially parallel to the axis of the propeller. Heat and pressure are applied to consolidate the material and to form a dense, homogeneous mass.

A propeller or other device embodying a 20 special fabric or woven material of substantially the type herein described and a phenolic condensation product or other binder which hardens and becomes substantially infusible and insoluble upon the application 25 of heat, is superior to similar devices made heretofore. The use of larger and stronger strands or cords increase both the elastic limit and the ultimate strength in the direction of such cords without sacrificing any 30 needed strength in other directions. A device, which is to be subjected to large strains and stresses in one direction with only minor stresses transversely to the said strains and stresses, when constructed in accordance with 35 my invention, will be considerably stronger than if made from ordinary fabric or other sheet material, particularly in the direction of maximum stresses.

Propellers employing the tightly twisted 40 cord fabric, while having a little less strength transversely, are approximately twice as strong longitudinally as those employing ordinary fabric used heretofore, while propellers employing the special fabric 45 embodying flat, loosely twisted cords have 2½ times the strength longitudinally of those employing ordinary fabric. The ultimate strength of the propellers embodying either of these special cord fabrics is 50 approximately the same, but the elastic limit of the one employing the loosely twisted cords is about 50% greater than the one employing the tightly twisted cords, both however, being distinctly superior to propellers made by previously well-known methods.

Obviously various changes in construction 60 of my new propeller may be made within the scope of my invention. For instance, I may utilize a suitable number of classes of strands placed in different directions to provide increased strength in such directions. Other binders may be substituted for the phenolic condensation product described. 65 Although I prefer to use this construction

in propellers it is obvious that it is equally well adapted to other application.

I claim as my invention:

1. A propeller comprising a fabric the strength of which is greater in one direction than in another and a phenolic condensation product as a binder. 70

2. A propeller comprising laminations of a material having a plurality of classes of strands, one of which predominates, and a 75 binder.

3. A propeller comprising laminations of a material having a plurality of classes of strands, one of which predominates, and a 80 binder which hardens and becomes substantially insoluble and infusible upon the application of heat.

4. A propeller comprising laminations of a material having a plurality of classes of strands, one of which predominates, and a 85 phenolic condensation product as a binder.

5. A propeller comprising a material having a plurality of classes of strands, the longitudinal strands of which predominate, and a phenolic condensation product as a 90 binder.

6. A propeller comprising a material having a plurality of classes of strands the longitudinal strands of which predominate, and a binder which hardens and becomes substantially insoluble and infusible upon the application of heat. 95

7. A propeller comprising laminations of a material having a plurality of classes of strands, the longitudinal strands of which predominate, and a phenolic condensation product as a binder. 100

8. A propeller comprising laminations of a material having a plurality of classes of strands, the longitudinal strands of which predominate, and a binder which hardens and becomes substantially insoluble and infusible upon the application of heat. 105

9. A propeller comprising a material having a plurality of classes of strands, the longitudinal strands of which are loose and flat twisted and substantially parallel to the longitudinal axis of the propeller, and a binder. 110

10. A propeller comprising a material having a plurality of classes of strands the longitudinal strands of which are loose and flat twisted and substantially parallel to the longitudinal axis of the propeller, and a binder which hardens and becomes substantially insoluble and infusible upon the application of heat. 115

11. A propeller comprising a material having a plurality of classes of strands, the longitudinal strands of which are loose and flat twisted and substantially parallel to the longitudinal axis of the propeller, and a phenolic condensation product as a binder. 120

12. A propeller comprising laminations of a material having a plurality of classes of 130

strands, the longitudinal strands of which are loose and flat twisted and substantially parallel to the longitudinal axis of the propeller, and a binder which hardens and becomes substantially insoluble and infusible upon the application of heat.

13. A propeller comprising a material having a plurality of classes of strands, the longitudinal strands of which are loose and flat twisted, and are substantially parallel to the longitudinal axis of the propeller and are relatively larger and more numerous than the transverse strands and a binder which hardens and becomes substantially insoluble and infusible upon the application of heat.

14. A propeller comprising laminations of a material having a plurality of classes of strands, the longitudinal strands of which

are loose and flat twisted, are substantially 20 parallel to the longitudinal axis of the propeller and are relatively larger and more numerous than the transverse strands, and a binder which hardens and becomes substantially insoluble and infusible upon the ap- 25 plication of heat.

15. A propeller comprising laminations of a material having a plurality of classes of strands the longitudinal strands of which are loose and flat twisted, are substantially 30 parallel to the longitudinal axis of the propeller and are relatively larger and more numerous than the transverse strands, and a phenolic condensation product as a binder.

In testimony whereof, I have hereunto 35 subscribed my name this 13th day of September 1923.

NOBLE S. CLAY.